

## 1

2,784,088

PHOTOGRAPHIC PAPER HAVING REDUCED  
PROCESSING CURLWilliam H. Griggs, Rochester, N. Y., assignor to Eastman  
Kodak Company, Rochester, N. Y., a corporation of  
New JerseyNo Drawing. Application November 8, 1954,  
Serial No. 467,631

6 Claims. (Cl. 96—85)

This invention concerns a method of treating photographic paper to eliminate or reduce the processing curl.

Early in the history of photographic paper manufacture, a slow rate of drying was used following coating with photographic emulsion. The curling characteristics of the paper thus prepared were not too unfavorable, particularly when the paper was stored in a place where there was not a great deal of variation in the relative humidity of the air in the place of storage. In recent years, however, the tendency has been to speed up the rate of drying of the emulsion coated paper, which has involved the use of elevated temperatures in those drying operations.

The cellulose fiber in the paper base of photographic paper and the gelatin in the emulsion layer thereof are both hygroscopic. They expand as they absorb water vapor at high humidity and contract as they desorb water vapor at low humidity. The rates of expansion and contraction of the two materials are not necessarily the same under a given set of conditions so that the stresses and strains set up in photographic paper often result in curl. This is especially true in the case of light-weight paper stocks such as those having a weight of 8-15 pounds per thousand square feet. When such paper is coated with an emulsion, often the stress in the emulsion layer is sufficiently great to result in face curl, or in other words, the curling of the paper towards the emulsion-coated side.

When wet photographic emulsion is applied to dry paper, some of the moisture from the emulsion penetrates the paper resulting in expansion of the paper base, while loss of water by the emulsion causes its contraction. Thus, the expansion of the paper and the contraction of the emulsion at that time sets up a balance of forces somewhat different from that obtained in the paper and the emulsion immediately prior to the absorption of water by the paper.

To avoid internal cracking of certain emulsions, sometimes the photographic emulsion is coated on the wire side of paper stock which provides a denser surface than the other side. As a result, the paper may curl towards the back (non-coated) side during processing when the processing solutions penetrate the paper and emulsion. The curl actually starts out as a face curl (towards the coated side) immediately upon immersion in the developer and then reverses to a back curl (towards the uncoated side) after about half the development time is up. At the time of development, the curl may be more extreme. It may become more pronounced during the balance of the processing cycle especially when a water rinse is used in place of short stop and when the wash water after fixing is on the alkaline side. In addition, the processing curl may tend to become more noticeable as the sensitized paper ages, usually reaching the worst point at about 6 months' age.

I have found that I can improve this process curl, especially with regard to the aging factor by coating a light size coat of a non-continuous film of polystyrene under the baryta on a wire side coated paper.

## 2

One object of my invention is to provide a photographic paper with reduced process curl. Another object is to provide a photographic paper coated on the wire side of the paper stock, which is relatively free from processing curl. An additional object is to provide a method for treating photographic paper, so that the paper will withstand wide variations in relative humidity without any appreciable curl.

The above objects are obtained by coating the wire side of photographic paper with a polystyrene resin dispersion in water containing about 10-15% solids. The coating is applied at about 2.5-4 grams per square meter and heat treated at a paper surface temperature of 275-320° F. for 5-10 seconds. Following the polystyrene coating, the paper is coated with a baryta-adhesive layer which is dried. A light-sensitive silver halide emulsion is superimposed over the baryta coating.

The following examples illustrate but are not intended to limit my invention.

Example I.—A roll of paper stock was coated on the wire side with three grams per square meter of a straight polystyrene resin dispersion in water containing from 10-15% solids. The coated stock was then heat treated at a paper surface temperature of 275-320° F. for 5-10 seconds using an infrared heater and was then given a 56 grams per square meter coat of baryta. The baryta-coated stock was sensitized with a silver bromide light-sensitive emulsion. The following curl results were obtained:

|                                                                                               |                  |
|-----------------------------------------------------------------------------------------------|------------------|
| 30                                                                                            | Equilibrium curl |
| Polystyrene coated paper                                                                      | —2.0             |
| Control sample, without the polystyrene coating,<br>but with the same silver bromide emulsion | —8.7             |

35 Equilibrium curl is the value obtained by measuring the change in distance across the arc of the curl from one edge of a 10 cm. disc of paper to the edge diametrically opposite. Therefore, if the paper were absolutely flat during processing there would be no change in this distance. However, when the paper curls this distance grows shorter. A value of 2.0, therefore, would denote that the paper has curled slightly, and the distance has shortened by 2 cm. The value of 8.7 cm. denotes a more pronounced curl, the distance being shortened by 8.7 cm. or that the edges are only 1.3 cm. apart. A negative sign (—) denotes curl towards the back, or uncoated side. The following results indicate the criticality of the weight of coating applied in regulating curl. The 2.5-4 grams per square meter coverage is quite critical as is shown by the following results.

|    |                               |                               |
|----|-------------------------------|-------------------------------|
| 40 | Coated paper samples:         | Equilibrium curl <sup>1</sup> |
| 55 | a. 1.5 grams per square meter | —5.5                          |
|    | b. 5.0 grams per square meter | —7.4                          |
|    | c. 3.0 grams per square meter | —3.3                          |
|    | d. Uncoated sample            | —9.1                          |

55 <sup>1</sup> 10 minutes in processing solutions.

60 Microscopic examination showed that the resin particles in the 3.0 grams per square meter coat were not completely fused, and therefore, the film was not continuous but full of very minute crevices which are of such a nature as not to permit very rapid solution penetration. The 1.5 gram coat was too thin to offer sufficient solution penetration. The cracks in the 5.0 clear coat had grown to sufficient size to appear as dry, cracked mud and to permit rapid solution penetration.

65 The heat treatment of the size coat described in Example I is essential to obtain partial resin particle fusion

with resulting optimum curl correction as is shown by the following data:

| Coated Paper Samples:                              | Equilibrium curl |
|----------------------------------------------------|------------------|
| a. 3. grams per square meter heated at 275-300° F. | -3.2             |
| b. 3. grams per square meter dried at 110° F. only | -6.5             |
| c. Untreated control                               | -7.1             |

A temperature of about 500-600° F. is necessary for complete resin particle fusion. It is obvious that the paper itself would not withstand these temperatures. The coating applied using 3 grams per square meter and heat treated at a temperature of 275-320° F. also offered good resistance to aging characteristics as follows:

|                                                                                | Equilibrium curl |
|--------------------------------------------------------------------------------|------------------|
| a. 3. grams per square meter, sensitized with a silver bromide emulsion, fresh | -2.0             |
| Accelerated aging <sup>1</sup>                                                 | -3.3             |
| 16 days incubation, 120° F., 35% relative humidity <sup>2</sup>                | -1.4             |
| b. Uncoated control sensitized with silver bromide emulsion, fresh             | -5.1             |
| Accelerated aging <sup>1</sup>                                                 | -9.1             |
| 16 days incubation at 120° F., 35% relative humidity <sup>2</sup>              | -10.5            |

<sup>1</sup> Formaldehyde fuming, equivalent of 6 months natural aging.  
<sup>2</sup> Equivalent of up to 2 years natural aging.

Regular print processing tests after two months natural aging verified this aging improvement.

*Example II.*—A roll of paper stock was coated in a manner similar to that described in Example I, except that hydroxy ether cellulose or similar thickener (1% solids based on total solution weight) was added to the polystyrene resin latex before coating.

This paper was subsequently baryta coated and sensitized with a silver bromide emulsion. Process curl tests showed even further improvement over the non-latex sized stock. The paper lay quite flat or had very slight face curl upon prolonged developing or in a water rinse after developing. The curl was comparable to that of face side coated stock.

A coating of polystyrene resin latex may be applied underneath the baryta layer on either the face side or the wire side of the paper depending upon the necessity of curl correction. Inasmuch as photographic paper curl is usually due to the shrinkage of the emulsion on drying, the coating would be applied under the baryta coating over which the photographic emulsion is superimposed. Almost all resin dispersions when coated on paper in which the percentage of the resin dispersion is bigger than 60% have been found to afford poor adhesive surfaces for other coatings such as gelatinous baryta coatings. However, I have found that using a coating of about 2.5-4 grams per square meter of polystyrene heat treated at a temperature of 275-320° F. that a discontinuous coating is obtained which permits the gelatinous baryta coating to adhere in spite of the rigid requirements of the photographic industry, particularly involv-

ing processing steps wherein the paper is immersed in alkaline solutions or in acid stop baths followed by heat drying.

It will be obvious to those skilled in the art that various paper stocks may be used and that the baryta-gelatin coating may be substituted by other coatings containing mineral fillers and adhesives such as casein, resin, latices and the like. Care must be taken, of course, that those mineral filler compositions be compatible both with the polystyrene and with the photographic emulsion.

I claim:

1. In a process for providing a photographic paper having a light-sensitive silver halide photographic emulsion coated over a baryta layer on the wire side of the paper, the step of first coating the paper under the baryta layer with 2.5-4 grams per square meter of an aqueous polystyrene resin latex and heat treating at a temperature of 275-320°.

2. A photographic paper containing three coatings over the paper base, the first comprising 2.5-4 grams per square meter of an aqueous polystyrene resin latex partly fused so that a discontinuous surface is formed, the second comprising a baryta layer and the third comprising a light-sensitive silver halide photographic emulsion.

3. A photographic paper containing three layers on the wire side of the paper base, the first comprising 2.5-4 grams per square meter of a polystyrene resin, partly fused so that a discontinuous surface is formed, the second comprising a baryta adhesive layer, and the third comprising a light-sensitive silver halide photographic emulsion.

4. In a photographic paper having a light-sensitive silver halide photographic emulsion coated over a baryta layer, a first coating on the paper under the baryta layer comprising 2.5-4 grams per square meter of polystyrene resin partly fused so that a discontinuous surface is formed.

5. In a photographic paper having a light-sensitive silver halide photographic emulsion coated over a baryta layer on the wire side of the paper, a first coating on the wire side of the paper under the baryta layer of 2.5-4 grams per square meter of polystyrene resin partly fused so that a discontinuous surface is formed.

6. A process for providing a photographic paper having improved processing curl, comprising coating the paper with 2.5-4 grams per square meter of a polystyrene resin latex, heat treating at a paper surface temperature of 275-320° F. for 5-10 seconds, coating with a baryta-adhesive coating composition, drying, and superimposing over the dried baryta layer a light-sensitive silver halide emulsion.

#### References Cited in the file of this patent

#### UNITED STATES PATENTS

2,366,723 Galley Jan. 9, 1943

#### OTHER REFERENCES

"Styrene" by Boundy-Boyer, published by Reinhold, New York, N. Y., 1952; pages 857-860.